

## UNITED STATES PATENT OFFICE

2,121,055

## CORROSION RESISTING IRON

Earle C. Smith, Cleveland Heights, and George T. Motok, Canton, Ohio, assignors to Republic Steel Corporation, Cleveland, Ohio, a corporation of New Jersey

No Drawing. Application January 6, 1937,  
Serial No. 119,264

5 Claims. (Cl. 75—125)

This invention relates to corrosion resisting compositions and more particularly to irons or steels with new and improved properties.

Irons and steels may be roughly divided into two classes on the basis of their resistance to corrosion. The first class includes those compositions which are highly resistant to corrosion, either because of the absence of impurities which cause corrosion or because of the presence of added elements which make them highly resistant to corrosion. An example of this class is stainless steel. The second class includes compositions which are only mildly resistant to corrosion, due to the presence of impurities, but which possess relatively long life under corroding influences by reason of a more or less uniform dispersion of the impurities in finely divided particles. Thus, while the metal corrodes, it does so slowly and uniformly as compared with the same metal in which the impurities are present in segregated form and where the corrosion is localized with the formation of pits or holes which soon make the article of little or no value. An example of this class is the iron of the Charles Patent No. 1,355,589.

The present invention is based on the discovery that nitrogen and phosphorus when present in the proper form and amounts, improve the properties of compositions of the second class, i. e., corrosion resisting irons or steels. We have found that, contrary to generally accepted belief, nitrogen in proper form and amount is not an element to be avoided, but in fact can be used to confer desirable characteristics on corrosion resisting irons having the fundamental composition of between about 0.01% and about 0.10% of carbon and between about 0.15% and about 1.5% of copper, with or without small quantities of other elements, such as molybdenum and manganese. The copper and carbon in this fundamental iron are distributed more or less uniformly in solution throughout the iron. When molybdenum is present, the dispersion of those elements is accentuated and other elements which may be present in small amounts, such as manganese, sulfur and silicon, are also similarly dispersed. Nickel may also be present in small amounts. We have found that when such an iron contains between about 0.005% and about 0.2% of nitrogen, preferably in the form of more or less stable metallic nitrides, the resistance of the iron to corrosion is considerably increased and its life under mildly corroding influences is correspondingly prolonged. We believe that these characteristics are traceable to the existence of nitrides of iron, and

possibly of other metals which are in the steel, in the form of minute, more or less uniformly distributed needles or particles which in themselves are highly resistant to corrosion and which serve as anchors to which may adhere iron oxide which forms during corrosion. These nitrides form a film which may be retained as a protective coating over the surface portions of the iron which are less resistant to corrosion. Such a film protects the iron from continued contact with the corroding agent and hence improves the resistance and prolongs the life of the iron. 5

We have also discovered that, contrary to previous generally accepted beliefs, phosphorus in proper amount is not an element to be avoided but in fact can be used to advantage to confer desirable characteristics on corrosion resisting irons of the foregoing fundamental composition and preferably containing about 0.005% and about 0.2% of nitrogen. The phosphorus should 10 be present in amounts between about 0.04% and about 0.5%. We believe that these new properties are traceable to the formation of a film on the surface of the iron during corrosive action. Apparently the phosphorus is converted into a 15 film-forming compound, which may include phosphates or phosphides when the iron is exposed to ordinary corroding influences. 20

The use of phosphorus, within the range specified, is particularly advantageous when the iron 30 contains nitrogen within the foregoing range, for the nitrogen apparently exerts a dispersing effect on the phosphorus and causes it to be more uniformly distributed throughout the iron.

In practicing the present invention an iron or 35 steel is made in the ordinary manner, as in an electric furnace or in an acid or basic open hearth or in a Bessemer furnace and/or converter, and contains between about 0.15% and about 1.5% of copper and between about 0.01% and about 0.10% of carbon, with or without between about 0.05% and about 0.55% of molybdenum and with or without between about 0.01% and about 0.50% manganese. Such iron or steel will ordinarily contain up to about 0.065% of phosphorus. When the melt is tapped into a ladle, a sufficient quantity of phosphorus or phosphorus-containing material is added to bring the total phosphorus content of the melt to between about 0.04% and about 0.50%. When the molten 50 metal is poured from the ladle into the ingot molds, nitrogen bearing material is thrown into the molds in amount sufficient to insure the presence of between about 0.005% and about 0.2% of nitrogen in the cold ingots. Alternatively the 55

nitrogen may be added when the phosphorus is added and both or either may be added to the molten metal in the furnace, in the ladle or in the molds.

5. Nitrogen carrying materials which have been found to be suitable for this purpose include nitrogen-bearing metallic materials, such as nitrides of copper or iron and cyanides of the alkali metals and alkaline earth metals. Urea or other organic compounds containing nitrogen may be used. The alkali and alkaline earth cyanides are quite useful. For example, calcium cyanamid is satisfactory both because of its nature and its low cost, and also because the residue remaining after it has decomposed and liberated nitrogen is beneficial to the iron. Such residues are inert under corroding conditions and hence may serve as an anchorage for films of iron oxide which protect underlying portions of the iron from corroding substances. The addition of about 5 lbs. of calcium cyanamid per ton of iron will carry a sufficient amount of nitrogen into the iron for the present purposes.

In order to insure retention in the iron of the desired amount of nitrogen, it is preferable to have ingredients present in the iron which will act as nitrogen fixers, i. e., elements which will readily combine with nitrogen liberated in the iron and form stable nitrides. Several metals have been found to be effective for this purpose, including titanium, vanadium, zirconium, columbium and tantalum. Silicon, aluminum, boron and beryllium are also good nitrogen fixers. Small amounts of one or more of these several elements may be used in amounts sufficient to retain in the iron nitrogen within the limits of from about 0.005% and about 0.2%.

Having thus described the invention so that those skilled in the art may practice the same, what we desire to secure by Letters Patent is defined in what is claimed.

What is claimed is:—

1. An iron article to be exposed during use to corroding conditions containing between about .01% and .10% carbon, between about .05% and

about .2% of nitrogen, between about .065% to about .5% of phosphorus, between .15%, and about 1.5% of copper, between about .05% and .55% of molybdenum and the ordinary small amounts of impurities normally present in iron, the remainder being iron.

2. An iron article to be exposed during use to corroding conditions, containing between about .01% and about .1% of carbon, between about .005% and about .2% of nitrogen, between about .04% and about .5% of phosphorus, between about .35% and about .65% of copper, impurities and molybdenum aggregating between about .30% and about .90%, the molybdenum ranging between about .05% and about .55% the remainder being iron.

3. An iron article to be exposed during use to corroding conditions containing between about .01% and about .1% of carbon, between about .007% and about .10% of nitrogen, between about .04% and about .5% of phosphorus, between about .35% and about .65% of copper, impurities and molybdenum aggregating between about .25% and about .35%, the molybdenum ranging between about .05% and about .15%, the remainder being iron.

4. An iron article to be exposed during use to corroding conditions containing between about .01% and about .1% of carbon, about .10% of nitrogen, about .5% of phosphorus, about .45% of copper, about .10% of molybdenum, the remainder consisting of iron containing small amounts of impurities.

5. An iron article to be exposed during use to corroding conditions composed of a low carbon, basic, open hearth iron containing between about .005% and about .2% of nitrogen, between about .04% and about .5% of phosphorus, between about .35% and about .65% copper, between about .3% and about .9% of ordinary impurities and molybdenum the molybdenum varying between about .05% and about .55%, the remainder being iron.

EARLE C. SMITH.  
GEORGE T. MOTOK. 45